

## UNITED STATES PATENT OFFICE

1,954,296

## WELDING ROD

James M. Keir, Bayside, N. Y., assignor to Oxweld  
Acetylene Company, a corporation of West  
Virginia

No Drawing. Application March 26, 1931,  
Serial No. 525,597

4 Claims. (Cl. 219—8)

This invention relates to welding rods for use in connection with metal deposition or welding and especially for use in connection with the carbon arc or metallic arc. It is among the 5 objects of the invention to devise a rod which will produce deposits which are composed essentially of carbon steel and are free from deleterious occlusions, to deposit the metal rapidly by using a large current in the arc, and to avoid 10 delays growing out of a need for playing the arc on the metal for refining purposes after the weld is formed.

Heretofore, readily oxidizable elements have been applied as coatings or cores to rods for arc 15 welding. The purpose of most rods of this kind was not to deposit a carbon steel. They were used to deposit alloy steels containing the elements used in the coating or core. Whether or not there was an excess of coating elements sufficient to produce an alloy deposit, I am not aware 20 of any of these rods which would deposit metal free from objectionable oxide inclusions, the deoxidizers when applied as a core or coating acting very inefficiently in the arc.

25 I have found that cleaner deposits can be obtained by properly choosing the deoxidizers and alloying them in proper proportion with iron or steel to form a welding rod or electrode; that by proceeding in this way I can deposit clean metal 30 even when the proportion of deoxidizers is not so great as to prevent their being largely eliminated during deposition; and that the deposited metal has the characteristics of carbon steel.

35 Deposits having the characteristics of carbon steel as used in the specification and claims means an alloy composed mainly of iron and containing carbon, manganese, silicon and minor impurities, the carbon being not more than about 0.5%, manganese not more than about 1.0% and silicon 40 not more than about 0.5%.

45 As deoxidizers, to be alloyed with iron to produce the rod material, I may use aluminum or titanium or both aluminum and titanium. Manganese and silicon are used in conjunction with the deoxidizers. Carbon may be present in quantities varying from insignificant traces up to about 0.6%, depending on the proportion of this element which is desired in the deposit.

50 As examples of suitable proportions of deoxidizing elements, I may state that about 0.25% to 4% of aluminum or titanium may be used, or a corresponding total of both of these elements. The silicon may range from about 0.5% to 1.5% and the manganese may range from 55 about 0.5% to 3%. Slightly greater variations

of silicon may be used with aluminum, namely from about 0.3% to 4.5%. In rods containing aluminum and the highest amounts of silicon, about 2.0% manganese is usually sufficient but more manganese can be used. The rods may 60 be varied to suit particular conditions, but for general purposes rods containing about 1.5% silicon, about 1% manganese, about 1% deoxidizing metal or metals (aluminum or titanium), and about 0.2% carbon give excellent results. 65

The rods of my invention are especially suitable for use with arcs carrying 200 amperes and upward to insure rapid deposition. With low currents it is necessary to play the arc to some extent on the deposited metal to refine the latter and burn out the alloying constituents. Arcs carrying 450 amperes give excellent results, and the current may be increased to 600 amperes or more. The higher the current, the more rapidly the non-ferrous components of the rod are 70 consumed and the more rapidly can the weld be completed. Larger proportions of deoxidizers are best suited for the heavier arcs. The rods of the invention produce voluminous slags and for the best results the heat generating properties 75 of electric arcs are required to keep the pools of deposited metal properly molten.

80 Arc welding with the described rods which contain the smaller amounts of silicon, manganese, aluminum and/or titanium is more rapid than 85 with the use of combustion torches when combustion torches are used under favorable welding conditions. With the use of the latter rods and combustion torches the most reliable results cannot be obtained with certainty in practice. Del- 90 eterious amounts of the alloy ingredients of the rods, oxide inclusions or weak joints are common causes of failure. With the largest amounts of alloy ingredients, combustion torches cannot be used. Increases in the alloy constituents of the 95 rods or less favorable welding conditions while applying the heat from combustion torches to the puddles of deposited metal, increase the chances of defective deposited metal or complete failure to form welds. The large amounts of 100 slag produced in welding with the rods of the invention always hinders the conduction of heat through the layer of slag when combustion torches are used.

105 In arc welding, the heat generated under the layer of slag by the action of the current, supplies the necessary heat to refine the metal which is violently oxidized during its passage through the arc, and the thick layer of slag avoids an excessive rate of oxidation after the deposit is 110

made. On the other hand, the oxidizable slag-forming and deoxidizing elements are present in kind, quantities and proportions which permit wide variations in other conditions usually present in welding, such as the thickness of plates, the sizes of the rods, and the sizes of the puddles of deposited metal.

With rods containing the lower proportions of silicon, manganese, aluminum and/or titanium, high welding speeds can be attained with the arc. When the amounts of these elements in the rods are below the minima set herein, uncertain results are obtained by reason of oxide inclusions. With the highest currents and the best welding conditions, silicon, manganese, aluminum and/or titanium may be increased somewhat beyond the highest limits specifically mentioned. It is to be understood that the statement of the upper limits of these elements in the specification and claims is intended to include such variations.

I claim:

25

100

30

105

35

110

40

115

45

120

50

125

55

130

60

135

65

140

70

145

75

150

1. A welding rod composed mainly of iron, having about 0.5% to 1.5% silicon, about 0.5% to 3.0% manganese, and about 0.25% to 4.0% of at least one of the following elements alloyed with the iron: aluminum, titanium, said rod containing carbon, the carbon not being in excess of about 0.5%.

2. A welding rod composed mainly of iron, having about 1.5% silicon, about 1.0% manganese, carbon about 0.2% and about 1.0% aluminum alloyed with the iron.

3. A welding rod composed mainly of iron, having about 0.3% to 4.5% silicon, about 0.5% to 3.0% manganese, carbon, the carbon not being in excess of about 0.5% and about 0.25% to 4.0% aluminum alloyed with the iron.

4. A welding rod composed mainly of iron, having about 1.5% silicon, about 2.0% to 3.0% manganese, carbon, the carbon not being in excess of about 0.5% and about 0.25% to 4.0% aluminum alloyed with the iron.

JAMES M. KEIR.

80

85

90

95